

## UNITED STATES PATENT OFFICE.

WILLIS M. PEIRCE AND EDMUND A. ANDERSON, OF PALMERTON, PENNSYLVANIA,  
ASSIGNORS TO THE NEW JERSEY ZINC COMPANY, OF NEW YORK, N. Y., A CORPO-  
RATION OF NEW JERSEY.

## MECHANICALLY-WORKED ZINC PRODUCT.

No Drawing.

Application filed February 9, 1928. Serial No. 253,213.

This invention relates to mechanically worked zinc products, such as rolled sheet or strip zinc, and has for its object the provision, as a new article of manufacture, of an improved zinc product of this nature. In its broader aspect, the invention contemplates the provision of a new zinc base alloy particularly adapted for the fabrication of superior mechanically worked zinc products.

10 In the production of rolled zinc, either by strip rolling or pack rolling, the properties of the finished rolled strips or sheets depend upon the composition of the zinc metal, as well as upon the rolling practice. Thus, 15 a substantially pure zinc metal, such as the well known Horsehead or other high grade brands, yields a very soft and ductile strip or sheet under suitable conditions of rolling. On the other hand, the more common grades 20 of zinc metal, such as the well known Prime Western or other lower grade brands, which are natural alloys of zinc, lead and cadmium containing higher percentages of cadmium than present in high grade zinc metal, yield 25 when rolled under appropriate conditions a stiffer and harder product than can be secured from a high grade zinc metal.

The stiffness of the strip or sheet rolled from the less pure grade of zinc gives for 30 certain purposes distinct advantages over the softer product rolled from high grade zinc. For example, one of the uses of rolled zinc is in the fabrication of corrugated sheets for roofing and siding purposes on buildings. 35 Here stiffness is of great importance, since it determines the gauge of zinc necessary to give adequate strength and resistance to plastic deformation or flow when the sheets are laid on the building purlins.

40 It is a recognized fact that zinc, like other metals of relatively low melting point, undergoes slow plastic deformation or flow when subjected continuously to loads as low as a quarter of the ultimate tensile strength 45 measured by ordinary tensile testing methods. For corrugated zinc sheets used as roofing, where the sheets must support snow loads and other loads continuously for considerable intervals, resistance to this plastic deformation 50 or flow is one of the important properties.

Our investigations and experiments have indicated that the amount of stiffening and increased resistance to plastic deformation or flow which can be secured through solid solu-

tion forming alloying elements, such as 55 cadmium, is limited, and we have, therefore, experimented with alloying elements which introduce a separate hardening constituent into the structure of the ultimate zinc base 60 alloy.

As a result of our investigations we have found that if copper and magnesium are added to zinc in suitable proportions, the 65 desired change in properties is secured to a very marked extent. This is presumably due 70 to the formation of a finely divided hard inter-metallic compound. Copper alone, in the amounts which we prefer to use, goes into solid solution and produces relatively little change in the properties of the zinc. Magnesium alone produces a distinct hardening. The combination of copper and magnesium in suitable relative proportions, produces a distinctly higher resistance to plastic deformation 75 or flow than is obtained in commercial zinc sheets rolled from the natural or usual zinc-cadmium-lead alloys.

We have found that the additions of copper and magnesium may be made to either 80 high grade zinc metal relatively free from lead and cadmium, or to lower grade zinc metal containing natural or usual amounts of cadmium and lead, with the production of improved zinc base alloys having the valuable properties for rolling or other mechanical 85 working. Copper and magnesium in suitable amounts produce a stiffening and hardening effect in all of the zinc base alloys to which we have added them regardless of the grade of zinc metal used as a base. Our investigations, however, indicate that best results 90 can be obtained when high grade, or substantially pure, zinc is employed.

We have found that the improved properties characteristic of the invention, that is 95 increased stiffness and hardness and increased resistance to plastic deformation or flow, can be secured by including in a zinc base alloy containing at least 92% of zinc, from 0.05 to 5% of copper and from .005 to 100 0.5% of magnesium, with not to exceed about 2% of such other metals as are naturally or otherwise included in the alloy. Preferably, however, the improved alloy of the invention contains a base of substantially pure zinc, from 0.5 to 2% of copper and from 0.005 to 105 0.1% of magnesium. We have secured excellent results with a zinc base alloy contain-

ing 97 to 99% of zinc, about 1% of copper, and about 0.01% of magnesium. Where maximum stiffness and hardness is desired, we prefer to use, in compounding the alloy, 5 high grade or substantially pure zinc metal, together with copper and magnesium in amounts just indicated.

The alloys of the invention may be compounded in any approved manner. In fabricating the improved mechanically worked zinc products of the invention, the alloy is cast into ingots of appropriate size and subsequently subjected to the contemplated mechanical working. Where the alloy is to be 15 rolled, the ingot is first given an appropriate number of passes through suitable roughing rolls, and may then be finished by strip rolling or pack rolling, as desired, in conjunction with such temperature treatment as may be 20 considered advantageous.

The following tables illustrate the improved properties of rolled sheet zinc made of the zinc base alloy of the invention:

| Alloy.              | Pb.  | Cd.   | Fe.   | Cu.   | Mg.   |
|---------------------|------|-------|-------|-------|-------|
| 1. Common metal mix | 0.75 | 0.10  | 0.02  | ----- | ----- |
| 2. High grade metal | 0.05 | 0.003 | 0.008 | ----- | ----- |
| 3. Of invention     | 0.75 | 0.10  | 0.02  | 1.0   | 0.01  |
| 4. Of invention     | 0.05 | 0.003 | 0.008 | 1.0   | 0.01  |
| 5. Of invention     | 0.05 | 0.003 | 0.008 | 1.4   | 0.007 |

| Alloy. | Gauge. | Hardness sclero-scope. | Temper. | Dynamic ductility. |
|--------|--------|------------------------|---------|--------------------|
| 1      | .032   | 23.5                   | 42      | .285               |
| 2      | .025   | 18-20                  | 34      | .315-.320          |
| 3      | .036   | 25-32                  | 46-51   | .270-.290          |
| 4      | .025   | 27-32                  | 46.5    | .250-.255          |
| 5      | .025   | 30-31                  | 51      | .200-.230          |

| Alloy. | Tensile strength. |               | Elongation. |               |                                                                              |
|--------|-------------------|---------------|-------------|---------------|------------------------------------------------------------------------------|
|        | With grain.       | Across grain. | % in 2 in.  |               | With grain; static load 8,000 lbs./sq. in. Time in hours to 5% elongation at |
|        |                   |               | With grain. | Across grain. |                                                                              |
| 1      | 27,700            | 40,700        | 30.5        | 26.0          | 58.3                                                                         |
| 2      | 19,000            | 22,200        | 37.6        | 40.0          | 46.6                                                                         |
| 3      | 36,400-           | 50,800-       | 10.8-       | 0.0-          | 3,310                                                                        |
| 4      | 44,900            | 56,500        | 15.0        | 2.5           | 201                                                                          |
| 5      | 37,800            | 49,900        | 26.3        | 1.5           | 5,550                                                                        |
|        | 46,700            | *             | 20.5        | *             | 4,520                                                                        |
|        |                   |               |             |               | 721. 242. 46.9 23.5                                                          |

\* Strip too narrow for cross grain test.

A study of these data will readily show the superior qualities of rolled sheet zinc of the invention over that of similar sheet zinc made directly from either high or low grade zinc. Thus, the elongation tests (which accelerate or speed up plastic deformation or flow) bring out the fact that plastic deformation 55 or flow is very substantially inhibited in the product of the invention as compared with products made directly from either high or low grade zinc. Tests conducted at 20° C. (with static loads of 8000 lbs./sq. in.) for example, indicate that in the case of common or

low grade zinc products (from alloy No. 1) it took 58.3 hours to secure a 5% elongation of the test specimen, whereas in the use of a product of the invention made from the same low grade zinc base (alloy No. 3) it took 3,310 70 hours to secure the same elongation.

Much the same situation obtains in the case of specimens made from high grade, or substantially pure, zinc. Whereas a 5% elongation was obtained in 46.6 hours with such a 75 specimen (alloy No. 2), it took 5,550 hours for the same elongation with a specimen of the invention alloyed with the same high grade zinc.

Zinc base alloys containing aluminum tend 80 to undergo intercrystalline oxidation. This is objectionable in alloys intended for rolling. For this reason the alloys of the invention are substantially free of aluminum.

The principles involved in the compound- 85 ing of zinc base alloys capable of being mechanically worked into wrought products possessing superior resistance to cold flow are disclosed in our copending patent application, Serial No. 346,493, filed March 12, 90 1929. The present invention is a species of that broad invention and is specifically directed to a zinc base alloy conforming to the principles underlying that broad invention.

We claim:

1. As a new article of manufacture, a mechanically worked zinc product made of a zinc base alloy substantially free of aluminum and containing not less than 92% of zinc, from 0.005 to 0.5% of magnesium, and from 0.05 100 to 5% of copper.

2. As a new article of manufacture, a mechanically worked zinc product made of a zinc base alloy containing 0.005-0.5% magnesium, and 0.05-5% copper, the remainder of 105 the alloy consisting of high grade zinc metal.

3. As a new article of manufacture, a mechanically worked zinc product made of a zinc base alloy substantially free of aluminum and, containing not less than 95% of zinc, 110 from 0.5 to 2% copper, and magnesium in amount not exceeding 0.5%.

4. As a new article of manufacture, a mechanically worked zinc product made of a zinc base alloy containing 0.5-2% copper and 115 0.005-0.1% magnesium, the remainder of the alloy consisting of high grade zinc metal.

5. As a new article of manufacture, a mechanically worked zinc product made of a zinc base alloy substantially free of aluminum 120 and containing not less than 95% of zinc, about 0.01% of magnesium, and about 1% of copper.

6. As a new article of manufacture, a mechanically worked zinc product made of a zinc base alloy containing about 0.01% magnesium and about 1% copper, the remainder of the alloy consisting of high grade zinc 125 metal.

7. A zinc base alloy substantially free of 130

aluminum and containing not less than 95% of zinc, from 0.005 to 0.5% of magnesium, and from 0.05 to 5% of copper.

8. A zinc base alloy containing 0.005-0.5% magnesium and 0.05-5% of copper, the remainder of the alloy consisting of high grade zinc metal.

9. A zinc base alloy substantially free of aluminum and containing not less than 95% of zinc, from 0.005 to 0.1% of magnesium, and from 0.05 to 2% of copper.

10. A zinc base alloy containing 0.005-0.1%

magnesium and 0.05-2% copper, the remainder of the alloy consisting of high grade zinc metal.

15

11. A zinc base alloy substantially free of aluminum and containing not less than 95% of zinc, about 0.01% of magnesium, and about 1% of copper.

In testimony whereof we affix our signatures.

WILLIS M. PEIRCE.  
EDMUND A. ANDERSON.